# EUROPEAN PATENT SPECIFICATION

(11) **EP 2 147 090 B1**
(45) Date of publication and mention of the grant of the patent: **22.12.2010**
(21) Application number: 08717230.0
(22) Date of filing: 28.02.2008
(51) Int. Cl.: C11D 3/40

(54) **TRIPHENYL METHANE AND XANTHENE PIGMENTS**
TRIPHENYLMETHAN- UND XANTHENPIGMENTE
PIGMENTS DE TRIPHÉNYL MÉTHANE ET DE XANTHÈNE

(30) Priority: 18.05.2007 EP 07108443
(43) Date of publication of application: 27.01.2010
(73) Proprietor: Unilever PLC, London EC4Y 0DY (GB); Unilever N.V., 3013 AL Rotterdam (NL)
(72) Inventor: BATCHELOR, Stephen, Norman, Bebington, Wirral Merseyside CH63 3JW (GB); BIRD, Jayne, Michelle, Bebington, Wirral Merseyside CH63 3JW (GB)
(74) Representative: Avila, David Victor
(86) International application number: PCT/EP2008/052446
(87) International publication number: WO 2008/141847

(56) References cited:
- EP-A- 0 184 888
- EP-A- 0 369 500
- WO-A-2006/041739
- GB-A- 1 313 180
- GB-A- 1 329 086
- US-A- 3 650 831
- US-A- 4 444 592
- US-A- 5 929 004

## Description

### FIELD OF INVENTION

The present invention concerns the use of organic pigments in laundry compositions.

### BACKGROUND OF INVENTION

Many garments yellow over multiple wash wear cycles, reducing the aesthetic value of the garment. In order to maintain the white appearance shading dyes may be used.

Colouring agents, when substantive to a fabric, are normally specific to a particular fibre type, for example cotton or polyester. WO 2006/032397 discloses the use of differing dye types in order to garments of differing fabrics and shade mixed garment fibres. EP 0184888 discloses coloured bleaching compositions which may contain heteropolyacid salts of triphenyl methane chromophores.

### SUMMARY OF INVENTION

We have found that blue and violet pigments based on triphenyl methane and xanthene chromphores with inorganic heteropolyacids efficiently deposit onto cotton, polyester and nylon. A consequence is that the pigments of the present invention may be used as a chromophore alone, i.e. without other blue/violet shading agents.

In one aspect the present invention provides laundry composition comprising between 0.00001 to 0.01 wt% of an organic pigment and 2 to 70 wt% of a surfactant, wherein the organic pigment is an inorganic heteropolyacid salt of a triphenyl methane or a xanthene moiety.

### DETAILED DESCRIPTION OF INVENTION

Organic pigments are described in 'Industrial Organic Pigments', Wiley VCH 2004 by W.Herbst and K.Hunger. Dyes are organic chemicals that are soluble in their application medium. Pigments are inorganic or organic particles that are insoluble in their application medium.

The present invention concerns pigments of the structure

Where the anion A⁻ is an inorganic heteropolyacid. The heteropolyacid is preferably selected from phosphomolybdic acid, phosphotungstic acid, phosphotungstomolybdic acid and silicomolybdic acid.

In the structures below the arrow indicates position of bonding to the pigment core structure.

Preferred pigments are triphenyl methane, when O is absent, or a xanthene moiety, when O is present and bonded at dashed lines, of the following form: wherein A- is an inorganic heteropolyacid;
R1 and R2 are independently selected from: hydrogen, C1-C6-alkyl and phenyl;
X is independently selected from the group consisting of: hydrogen, C1-C6-alkyl and benzyl;
Ar is selected from: wherein Y is hydrogen, C1-C6-alkyl or benzyl; wherein R1 and R2 are as defined above; R₁ is hydrogen, C1-C6-alkyl, or phenyl; R₄ is hydrogen, C1-C6-alkyl, or phenyl.

The R₁ and R₂ groups are independently selected from hydrogen, methyl and ethyl groups, preferably methyl and ethyl. Preferably the R1 groups are same. Preferably the R1 groups are the same and the R2 groups are the same.

X is selected from hydrogen and methyl, preferably hydrogen.

The central oxygen shown with dashed bonds is optional; the triphenyl methane pigments are most preferred.

When the central Oxygen atom is present, then the Ar group is preferably in which Y is selected from hydrogen, methyl and ethyl groups.

In the absence of the central oxygen the Ar group is preferably selected from: where the R₃ is selected from hydrogen, methyl or ethyl, preferably hydrogen and R₄ is selected from methyl, ethyl or phenyl. The amine substituted phenyl group is preferred rather than the naphthyl.

Preferred pigments are pigment violet 3, pigment violet 27, pigment violet 39, pigment violet 1, pigment violet 1:1, pigment violet 1:2, pigment blue 1, pigment blue 1:2, pigment blue 1:3 pigment blue 2, pigment blue 10, pigment blue 10:1, pigment blue 11, pigment blue 14 and pigment blue 62.

Most preferably pigment violet 3, pigment violet 27, pigment violet 39 and pigment blue 14.

It is most preferred that pigments are used alone and not in combination with other blue or violet shading dyes. In this regard the laundry composition contains less than 0.00004 wt% of a blue or violet shading dye and is preferably devoid of such.

### SURFACTANT

The composition comprises between 2 to 70 wt% of a surfactant, most preferably 10 to 30 wt %. In general, the nonionic and anionic surfactants of the surfactant system may be chosen from the surfactants described "Surface Active Agents" Vol. 1, by Schwartz & Perry, Interscience 1949, Vol. 2 by Schwartz, Perry & Berch, Interscience 1958, in the current edition of "McCutcheon's Emulsifiers and Detergents" published by Manufacturing Confectioners Company or in "Tenside-Taschenbuch", H. Stache, 2nd Edn., Carl Hauser Verlag, 1981. Preferably the surfactants used are saturated.

Suitable nonionic detergent compounds which may be used include, in particular, the reaction products of compounds having a hydrophobic group and a reactive hydrogen atom, for example, aliphatic alcohols, acids, amides or alkyl phenols with alkylene oxides, especially ethylene oxide either alone or with propylene oxide. Specific nonionic detergent compounds are C₆ to C₂₂ alkyl phenol-ethylene oxide condensates, generally 5 to 25 EO, i.e. 5 to 25 units of ethylene oxide per molecule, and the condensation products of aliphatic C₈ to C₁₈ primary or secondary linear or branched alcohols with ethylene oxide, generally 5 to 40 EO.

Suitable anionic detergent compounds which may be used are usually water-soluble alkali metal salts of organic sulphates and sulphonates having alkyl radicals containing from about 8 to about 22 carbon atoms, the term alkyl being used to include the alkyl portion of higher acyl radicals. Examples of suitable synthetic anionic detergent compounds are sodium and potassium alkyl sulphates, especially those obtained by sulphating higher C₈ to C₁₈ alcohols, produced for example from tallow or coconut oil, sodium and potassium alkyl C₉ to C₂₀ benzene sulphonates, particularly sodium linear secondary alkyl C₁₀ to C₁₅ benzene sulphonates; and sodium alkyl glyceryl ether sulphates, especially those ethers of the higher alcohols derived from tallow or coconut oil and synthetic alcohols derived from petroleum. The preferred anionic detergent compounds are sodium C₁₁ to C₁₅ alkyl benzene sulphonates and sodium C₁₂ to C₁₈ alkyl sulphates. Also applicable are surfactants such as those described in EP-A-328 177 (Unilever), which show resistance to salting-out, the alkyl polyglycoside surfactants described in EP-A-070 074, and alkyl monoglycosides.

Preferred surfactant systems are mixtures of anionic with nonionic detergent active materials, in particular the groups and examples of anionic and nonionic surfactants pointed out in EP-A-346 995 (Unilever). Especially preferred is surfactant system that is a mixture of an alkali metal salt of a C₁₆ to C₁₈ primary alcohol sulphate together with a C₁₂ to C₁₅ primary alcohol 3 to 7 EO ethoxylate.

The nonionic detergent is preferably present in amounts greater than 10%, e.g. 25 to 90 wt % of the surfactant system. Anionic surfactants can be present for example in amounts in the range from about 5% to about 40 wt % of the surfactant system.

In another aspect which is also preferred the surfactant may be a cationic such that the formulation is a fabric conditioner.

### CATIONIC COMPOUND

When the present invention is used as a fabric conditioner it needs to contain a cationic compound.

Most preferred are quaternary ammonium compounds.

It is advantageous if the quaternary ammonium compound is a quaternary ammonium compound having at least one C₁₂ to C₂₂ alkyl chain.

It is preferred if the quaternary ammonium compound has the following formula: in which R¹ is a C₁₂ to C₂₂ alkyl or alkenyl chain; R², R³ and R⁴ are independently selected from C₁ to C₄ alkyl chains and X⁻ is a compatible anion. A preferred compound of this type is the quaternary ammonium compound cetyl trimethyl quaternary ammonium bromide.

A second class of materials for use with the present invention are the quaternary ammonium of the above structure in which R¹ and R² are independently selected from C₁₂ to C₂₂ alkyl or alkenyl chain; R³ and R⁴ are independently selected from C₁ to C₄ alkyl chains and X⁻ is a compatible anion.

A detergent composition according to claim 1 in which the ratio of (ii) cationic material to (iv) anionic surfactant is at least 2:1.

Other suitable quaternary ammonium compounds are disclosed in EP 0 239 910 (Proctor and Gamble).

It is preferred if the ratio of cationic to nonionic surfactant is from 1:100 to 50:50, more preferably 1:50 to 20:50.

The cationic compound may be present from 1.5 wt % to 50 wt % of the total weight of the composition. Preferably the cationic compound may be present from 2 wt % to 25 wt %, a more preferred composition range is from 5 wt % to 20 wt %.

The softening material is preferably present in an amount of from 2 to 60% by weight of the total composition, more preferably from 2 to 40%, most preferably from 3 to 30% by weight.

The composition optionally comprises a silicone.

### FLUORESCENT AGENT

The composition preferably comprises a fluorescent agent (optical brightener). Fluorescent agents are well known and many such fluorescent agents are available commercially. Usually, these fluorescent agents are supplied and used in the form of their alkali metal salts, for example, the sodium salts. The total amount of the fluorescent agent or agents used in the composition is generally from 0.005 to 2 wt %, more preferably 0.01 to 0.1 wt %. Preferred classes of fluorescer are: Di-styryl biphenyl compounds, e.g. Tinopal (Trade Mark) CBS-X, Di-amine stilbene di-sulphonic acid compounds, e.g. Tinopal DMS pure Xtra and Blankophor (Trade Mark) HRH, and Pyrazoline compounds, e.g. Blankophor SN. Preferred fluorescers are: sodium 2 (4-styryl-3-sulfophenyl)-2H-napthol[1,2-d]trazole, disodium 4,4'-bis{[(4-anilino-6-(N-methyl-N-2 hydroxyethyl) amino 1,3,5-triazin-2-yl)]amino}stilbene-2-2' disulfonate, disodium 4,4'-bis{[(4-anilino-6-morpholino-1,3,5-triazin-2-yl)]amino} stilbene-2-2' disulfonate, and disodium 4,4'-bis(2-sulfoslyryl)biphenyl.

### PERFUME

Preferably the composition comprises a perfume. The perfume is preferably in the range from 0.001 to 3 wt %, most preferably 0.1 to 1 wt %. Many suitable examples of perfumes are provided in the CTFA (Cosmetic, Toiletry and Fragrance Association) 1992 International Buyers Guide, published by CFTA Publications and OPD 1993 Chemicals Buyers Directory 80th Annual Edition, published by Schnell Publishing Co.

### Examples

### Pigment Violet 1:2

Phosphotungstomolybdic acid salt of

### Pigment violet 3

Phosphotungstomolybdic acid salt of

### Pigment Violet 39

Phosphomolybdic salt of

### Pigment Blue 1

Phosphotungstomolybdic acid salt of Pigment violet 14 is an inorganic pigment based on (CO)₃(PO₄)₂

### Example 1

Pigments were tested for shading benefit by washing cotton, polyester-cotton, polyester, nylon-elastane fabric together at room temperature, in 2.0g/L of a base washing powder which contained: 18% NaLAS, 73% salts (silicate, sodium tri-poly-phosphate, sulphate, carbonate), 3% minors including fluorescer and enzymes, remainder.impurities and water. A liquor to cloth of with a 30:1 was used, the wash lasted for 30 mins, and were conducted with and without the addition of 500 part per billion of the pigment. Pigments were added from a 0.005 wt% solution in ethanol. All pigments were used as received. Following the wash, the cloths were rinses then drying. The colour of the cloth was then assessed using a reflectometer (UV excluded for all measurements) and expressed as the ΔE value relative to cloth washed without pigment. The pigments tested and ΔE values are given in the table below.

All the triphenyl methane and xanthene based pigments showed good deposition over the range of the fabrics. In contrast, the inorganic pigment violet 14 shows very low deposition on these fabrics.

| Pigment | WC | KC | WP | WPC | NE |
|---|---|---|---|---|---|
| violet 1:2 | 2.8 | 2.7 | 0.4 | 1.2 | 1.5 |
| Violet 3 | 0.9 | 1.0 | 0.2 | 1.1 | 1.0 |
| Violet 39 | 0.4 | 1.2 | 0.3 | 1.4 | 1.7 |
| Blue 1 | 2.1 | 1.6 | 1.0 | 1.5 | 1.8 |
| Violet 14 | 0.2 | 0.1 | 0.1 | 0.3 | 0.3 |

| | | | | | |
|---|---|---|---|---|---|
| Fabric codes: WC = woven cotton KC = knitted cotton WP = woven polyester WPC = 65/35 woven polyester cotton NE = 90/10 nylon elastane | | | | | |

## Claims

1. A laundry composition comprising between 0.00001 to 0.01 wt% of an organic pigment and 2 to 70 wt% of a surfactant, wherein the organic pigment is an inorganic heteropolyacid salt of a triphenyl methane or a xanthene moiety.

2. A laundry composition according to claim 1, wherein the triphenyl methane, when O is absent, or a xanthene moiety, when O is present and bonded at dashed lines, is of the following form: wherein A- is an inorganic heteropolyacid;
R1 and R2 are independently selected from: hydrogen, C1-C6-alkyl and phenyl;
X is independently selected from the group consisting of: hydrogen, C1-C6-alkyl and benzyl;
Ar is selected from: wherein Y is hydrogen, C1-C6-alkyl or benzyl; wherein R1 and R2 are as defined above; R₃ is hydrogen, C1-C6-alkyl, or phenyl; R₄ is hydrogen, C1-C6-alkyl, or phenyl.

3. A laundry composition according to claim 2, wherein R1 and R2 are independently selected from: hydrogen, methyl and ethyl;
X is independently selected from the group consisting of: hydrogen and methyl;
Ar, when the organic pigment is a xanthene moiety is and Y is selected from hydrogen, methyl and ethyl group;
Ar, when the organic pigment is a triphenyl methane moiety, is selected from the group consisting of: wherein R1 and R2 are as defined above;
R₃ is selected from: hydrogen, methyl or ethyl; and,
R₄ is selected from methyl, ethyl or phenyl.

4. A laundry composition according to any preceding claim, wherein substituents R1 are same and substituents R2 are same.

5. A laundry composition according to any preceding claim, wherein the organic pigment is a triphenyl methane pigment.

6. A laundry composition according to claim 1, wherein the organic pigment is selected from the group consisting of: pigment violet 3, pigment violet 27, pigment violet 39, pigment violet 1, pigment violet 1:1, pigment violet 1:2, pigment blue 1, pigment blue 1:2, pigment blue 1:3 pigment blue 2, pigment blue 10, pigment blue 10:1, pigment blue 11, pigment blue 14 and pigment blue 62.

7. A laundry composition according to claim 6, wherein the organic pigment is selected from the group consisting of: pigment violet 3, pigment violet 27, pigment violet 39 and pigment blue 14.

8. A laundry composition according to any preceding claim, wherein the inorganic heteropolyacid is selected from the group consisting of: phosphomolybdic acid, phosphotungstic acid, phosphotungstomolybdic acid and silicomolybdic acid.

9. A domestic method of treating a textile, the method comprising the steps of:
(i) treating a textile with an aqueous solution of the pigment as defined in any one of claims 1 to 8, the aqueous solution comprising from 1 ppb to 1 ppm of the pigment, and, from 0.2 g/L to 3 g/L of a surfactant; and,
(ii) rinsing and drying the textile.

10. A method according to claim 9, wherein the pigment is present from 10 ppb to 200 ppb.

## Patentansprüche

1. Waschmittel-Zusammensetzung, umfassend zwischen 0,00001 und 0,01 Gewichts-% eines organischen Pigments und 2 bis 70 Gewichts-% eines Tensids, wobei das organische Pigment ein anorganisches Heteropolysäuresalz einer Triphenylmethan- oder einer Xanthen-Gruppierung ist.

2. Waschmittel-Zusammensetzung nach Anspruch 1, wobei die Triphenylmethan-Gruppierung, wenn O nicht vorhanden ist, oder eine Xanthen-Gruppierung, wenn O vorhanden ist und an den gestrichelten Linien gebunden ist, die folgende Formel hat: worin A- eine anorganische Heteropolysäure ist;
R1 und R2 unabhängig ausgewählt sind aus: Wasserstoff, C1-C6-Alkyl und Phenyl;
X unabhängig ausgewählt ist aus der Gruppe, bestehend aus: Wasserstoff, C1-C6-Alkyl und Benzyl;
Ar ausgewählt ist: worin Y Wasserstoff,
C1-C6-Alkyl und Benzyl ist; worin R1 und R2 wie oben definiert sind; R3 Wasserstoff, C1-C6-Alkyl oder Phenyl ist; R₄ Wasserstoff, C1-C6-Alkyl oder Phenyl ist.

3. Waschmittel-Zusammensetzung nach Anspruch 2, wobei R1 und R2 unabhängig ausgewählt sind aus: Wasserstoff, Methyl und Ethyl;
X unabhängig ausgewählt ist aus der Gruppe, bestehend aus: Wasserstoff und Methyl;
Ar, wenn das organische Pigment eine Xanthen-Gruppierung ist, ist, und Y aus Wasserstoff, Methyl- und Ethyl-Gruppe ausgewählt ist;
Ar, wenn das organische Pigment eine Triphenylmethan-Gruppierung ist, aus der Gruppe, bestehend aus worin R1 und R2 wie oben definiert sind, ausgewählt ist;
R₃ aus: Wasserstoff, Methyl oder Ethyl, ausgewählt ist und
R₄ aus Methyl, Ethyl und Phenyl ausgewählt ist.

4. Waschmittel-Zusammensetzung nach einem vorangehenden Anspruch, wobei die Substituenten R1 gleich sind und die Substituenten R2 gleich sind.

5. Waschmittel-Zusammensetzung nach einem vorangehenden Anspruch, wobei das organische Pigment ein Triphenylmethan-Pigment ist.

6. Waschmittel-Zusammensetzung nach Anspruch 1, wobei das organische Pigment ausgewählt ist aus der Gruppe, bestehend aus: Pigment Violet 3, Pigment Violet 27, Pigment Violet 39, Pigment Violet 1, Pigment Violet 1:1, Pigment Violet 1:2, Pigment Blue 1, Pigment Blue 1:2, Pigment Blue 1:3, Pigment Blue 2, Pigment Blue 10, Pigment Blue 10:1, Pigment Blue 11, Pigment Blue 14 und Pigment Blue 62.

7. Waschmittel-Zusammensetzung nach Anspruch 6, wobei das organische Pigment aus der Gruppe, bestehend aus Pigment Violet 3, Pigment Violet 27, Pigment Violet 39 und Pigment Blue 14, ausgewählt ist.

8. Waschmittel-Zusammensetzung nach einem vorangehenden Anspruch, wobei die anorganische Heteropolysäure aus der Gruppe, bestehend aus Phosphomolybdänsäure, Phosphowolframsäure, Phosphowolframatomolybdänsäure und Silicomolybdänsäure, ausgewählt ist.

9. Verfahren zur häuslichen Behandlung einer Textilie, wobei das Verfahren die folgenden Schritte umfasst:
(i) Behandeln einer Textilie mit einer wässrigen Lösung des Pigments, wie in einem der Ansprüche 1 bis 8 definiert, wobei die wässrige Lösung 1 ppb bis 1 ppm des Pigments und 0,2 g/l bis 3 g/l eines Tensids umfasst, und
(ii) Spülen und Trocknen der Textilie.

10. Verfahren nach Anspruch 9, wobei das Pigment mit 10 ppb bis 200 ppb vorliegt.

## Revendications

1. Composition pour le lavage du linge comprenant entre 0,00001 et 0,01 % en poids d'un pigment organique et de 2 à 70 % en poids d'un tensioactif, dans laquelle le pigment organique est un sel d'hétéropolyacide inorganique d'un fragment triphénylméthane ou xanthène.

2. Composition pour le lavage du linge selon la revendication 1, dans laquelle le triphényl-méthane, quand O est absent, ou un fragment xanthène, quand O est présent et lié comme indiqué par les pointillés, est sous la forme suivante : dans laquelle A⁻ est un hétéropolyacide inorganique ;
R₁ et R₂ sont indépendamment choisis parmi : hydrogène, alkyle en C₁-C₆ et phényle ;
X est indépendamment choisi dans le groupe constitué par : hydrogène, alkyle en C₁-C₆ et benzyle ;
Ar est choisi parmi : où Y est hydrogène, alkyle en C₁-C₆ ou benzyle ; où R₁ et R₂ sont tels que définis ci-dessus ; R₃ est hydrogène, alkyle en C₁-C₆, ou phényle ; R₄ est hydrogène, alkyle en C₁-C₆, ou phényle.

3. Composition pour le lavage du linge selon la revendication 2, dans laquelle R₁ et R₂ sont indépendamment choisis parmi : hydrogène, méthyle et éthyle ;
X est indépendamment choisi dans le groupe constitué par : hydrogène et méthyle ;
Ar, quand le pigment organique est un fragment xanthène, est et Y est choisi parmi un atome d'hydrogène, un groupe méthyle et éthyle ;
Ar, quand le pigment organique est un fragment triphénylméthane, est choisi dans le groupe constitué par : où R₁ et R₂ sont tels que définis ci-dessus ;
R₃ est choisi parmi : hydrogène, méthyle ou éthyle ; et
R₄ est choisi parmi méthyle, éthyle ou phényle.

4. Composition pour le lavage du linge selon l'une quelconque des revendications précédentes, dans laquelle les substituants R₁ sont identiques et les substituants R₂ sont identiques.

5. Composition pour le lavage du linge selon l'une quelconque des revendications précédentes, dans laquelle le pigment organique est un pigment triphényl-méthane.

6. Composition pour le lavage du linge selon la revendication 1, dans laquelle le pigment organique est choisi dans le groupe constitué par : le pigment violet 3, le pigment violet 27, le pigment violet 39, le pigment violet 1, le pigment violet 1:1, le pigment violet 1:2, le pigment bleu 1, le pigment bleu 1:2, le pigment bleu 1:3, le pigment bleu 2, le pigment bleu 10, le pigment bleu 10:1, le pigment bleu 11, le pigment bleu 14 et le pigment bleu 62.

7. Composition pour le lavage du linge selon la revendication 6, dans laquelle le pigment organique est choisi dans le groupe constitué par : le pigment violet 3, le pigment violet 27, le pigment violet 39 et le pigment bleu 14.

8. Composition pour le lavage du linge selon l'une quelconque des revendications précédentes, dans laquelle l'hétéropolyacide inorganique est choisi dans le groupe constitué par : l'acide phosphomolybdique, l'acide phosphotungstique, l'acide phosphotungsto-molybdique et l'acide silico-molybdique.

9. Procédé domestique de traitement d'un textile, le procédé comprenant les étapes consistant à :
(i) traiter un textile avec une solution aqueuse du pigment telle que définie dans l'une quelconque des revendications 1 à 8, la solution aqueuse comprenant de 1 ppb à 1 ppm de pigment et de 0,2 à 3 g/l de tensioactif ; et
(ii) rincer et sécher le textile.

10. Procédé selon la revendication 9, dans lequel le pigment est présent à raison de 10 à 200 ppb.
